

Nov. 29, 1927.

1,651,136

G. E. LANG

METHOD OF PRODUCING WOOD GRAIN SURFACES

Filed Dec. 20. 1926



FIG.- 2



FIG.- 1

Inventor

George E. Lang

By Bates, Macklin, Dolnick & Pearce

Attorneys

Patented Nov. 29, 1927.

1,651,136

# UNITED STATES PATENT OFFICE.

GEORGE E. LANG, OF DETROIT, MICHIGAN, ASSIGNOR TO OXFORD VARNISH CORPORATION, OF DETROIT, MICHIGAN, A CORPORATION OF MICHIGAN.

## METHOD OF PRODUCING WOOD GRAIN SURFACES.

Application filed December 20, 1926. Serial No. 155,906.

This invention is directed to improvements in the method of obtaining the reproduction of a wood grain on hard surfaces and the general object thereof is the provision of a process for obtaining an increase in depth of tone and color contrast while effecting a more accurate blending of the colors and thus more accurately simulating the appearance of a natural wood grain.

10 More specifically, my invention is concerned with improvements in the process of reproducing wood grain effects by the use of the photogravure process.

Further objects of my invention will be 15 come apparent from the hereinafter set forth description. The essential characteristics of my novel graining process are summarized in the claims.

I show in the drawings in Fig. 1, an enlarged cross section of an article, the surface of which has a wood grain finish applied thereto and in Fig. 2 I show a similar cross section of a material having a hard surface and having a wood grain appearance effected thereon by a process of a modified form.

My invention contemplates the provision of an improved method of reproducing the appearance of a natural wood grain on a hard surface such as metallic sheeting, wherein the actual grain is obtained by the use of a photogravure plate or roll and a transfer roll. The photogravure film or plate comprises an etched negative of a wood panel, the grained surface of which is to be simulated. The preparation of such plates or rolls is set forth in Patent No. 1,548,465 issued August 4, 1925 on the application of James P. Henry.

40 I have found however, that the desired result cannot be obtained by the mere application of a wood grain transfer to the surface to be grained without considerable attention being directed to the combining of the ground colors and the color of the transfer ink or pigment in an accurately predetermined manner and even when such care is taken, the full reproductive effect of the transfer may not be apparent except when 45 the grained surface is viewed from a direction normal to the grained surface. This is due to a considerable extent, to the glare set up by the finishing material which is usually applied in the nature of a varnish or lacquer, 50 to protect the graining pigment.

By combining in the ground color, or by applying over the ground color, a secondary ground coating which carries in its composition a flaked material such as powdered bronze or aluminum flake which is not entirely submerged or concealed by the other constituents of the pigment composition in which it is mixed, a tonal depth is imparted to the finished product which may be accounted for by the action of the minute flaked surfaces in breaking up the uniformity of the light refraction of the varnish or lacquer which constitutes the final coating of the grained surface.

60 The use of such material in the manner I will hereinafter set forth, greatly assists in bringing about variations in the tonal depth of the graining transfer and is also highly effective in reproducing ground colors of certain natural woods when stained or 65 grained and treated with a varnish or lacquer. In other words variation in the high and low tone contrasts is now obtained, which heretofore has not been believed possible.

70 Referring to the drawings in Fig. 1, L represents a cross section of a metallic panel or a panel formed of other hard material to be grained. After proper cleaning of the 75 surface thereof, I apply a base pigment F which may constitute a ground color and filler. After proper drying of the ground color I then apply a layer or coating G which may comprise a colored lacquer, paint or varnish and which will have a dull or 80 unglossed surface when dry, the color of this coating G corresponding to the general ground color of the natural grain wood to be simulated. Over the full dry coating G, 85 is then applied a pigment layer H carrying in its composition powdered bronze or powdered aluminum or similar flaked material; the mixture being such that the flaked material will not segregate or separate out of the mixture and rise to the surface but will 90 remain homogeneously suspended when the layer H becomes dry. The flaked surface is then visibly submerged somewhat by a semi-transparent paint or lacquer coating I.

95 The surface to be grained is now in condition to receive the transfer of the wood grain pattern from the etched photogravure plate and this is represented by the layer J in Fig. 1. It will be noted that this layer 100 varies in thickness throughout and that the 105 110

cross section completely disappears at certain points as indicated at M. For a more clear understanding of the obtaining of this transfer, reference can be made to the patent 5 hereinbefore referred to. The graining paste or pigment comprising the layer J however, should correspond as closely as possible in color to the natural graining color of the wood being simulated. After proper 10 drying of the transfer I then apply a protective coating of varnish or lacquer K.

A surface finish in the manner just described will have a velvet appearance simulating the appearance, for example, of a 15 natural bird's eye maple when properly grained and surfaced and imparts a submerged sheen or luster to the finished surface and without over-prominence of the flaked material.

20 In Fig. 2 I show a modified method of obtaining the surfacing effect illustrated in Fig. 1. The ground color A is first applied and then over the ground color I apply a transparent varnish or lacquer which also 25 carries the flaked material mixed therein. Over the ground color I then apply on a semitransparent color pigment C. I then apply the transfer D and subsequently protect the transfer by a finish coating of lacquer or varnish E.

It is to be understood that flaked material 30 may be combined in any one of the coatings underlying the transfer, in a manner to partly submerge the full visible effect thereof and I accordingly consider the use of the flaked material in an underlying coating upon which a transfer is applied within the scope of the novelty of my invention.

I claim:

40 1. The method of obtaining a wood grain finish on a hard surface which includes the steps of coating the surface to be grained

with a ground color pigment or filler, apply a dull drying coating of lacquer or varnish to the ground coating, applying a flaked 45 pigment to the dull dry coating, thereafter applying a semi-transparent paint or lacquer to the flaked coating, then applying to the semi-transparent coating of paint or lacquer a wood grain transfer pattern and finally 50 applying to the transfer a transparent varnish or lacquer.

2. The method of reproducing the wood grain effect on a surface comprising coating the surface with a ground color, applying to 55 the ground color coating a transparent varnish or lacquer containing a flaked pigment, applying a semi-transparent color coating to the last named coating, then applying a wood grain transfer to the semi-transparent 60 color coating and finally applying a protective transparent lacquer or varnish to the transfer.

3. The method of obtaining a wood grain finish on a hard surface which includes the 65 application of a ground color pigment and a flaked pigment to underlie a wood grain transfer pattern and then applying to the transfer a transparent varnish or lacquer.

4. The method of reproducing a wood grain effect which includes the application 70 of a wood grain transfer pattern to a surface which has been previously covered with a flaked pigment wherein the flakes of the pigment remain visibly exposed and finally 75 applying a protective transparent lacquer or varnish to the transfer whereby the pigment flakes remain visibly exposed in varying degree through the less dense regions of the transfer.

In testimony whereof, I hereunto affix my signature.

GEORGE E. LANG.